

## UNITED STATES PATENT OFFICE

2,385,765

## TEXTILE FINISHING

Jack T. Thurston, Cos Cob, Conn., assignor to  
American Cyanamid Company, New York, N. Y.  
a corporation of Maine

No Drawing. Application August 30, 1941,  
Serial No. 409,112

16 Claims. (Cl. 117—139.5)

This invention relates to the treating and finishing of textiles and textile-forming materials such as cotton, linen, wool, viscose, silk, cellulose acetate, spun rayon and the like. More particularly, the invention relates to textile finishing processes, to finishing compositions and to textiles finished with compositions consisting of or containing higher alkyl guanamines and their aldehyde condensation products, as will be described.

A wide variety of softening agents, lubricants, creaseproofing agents and waterproofing agents have heretofore been applied to textile threads and fibers. The treatment of textiles for these and similar purposes such as shrinkproofing is known as textile finishing, and the agents employed are known as textile finishing agents. It is a principal object of the present invention to provide a new class of textile finishing agents having improved softening, waterproofing and other properties, and to provide new and improved textile finishing processes employing such materials. A further important feature of the invention resides in the provision of cotton, linen, wool, silk, cellulose ester and other yarns, threads or fabrics finished with compositions containing higher alkyl guanamines and their reaction products and having improved water-resistance and a more desirable hand.

I have found that the higher alkyl guanamines, in which the alkyl group attached to the 2-carbon atom of the triazine nucleus contains at least 7 carbon atoms with or without other substituents in addition to hydrogen, possess remarkable properties when applied to textiles of the above and similar classes. Many of these guanamines, as such, have softening and lubricating properties for certain textile fibers, notably cotton, and they also impart water-repellent properties to a marked degree. Moreover, these water-repellent properties may be greatly enhanced by further reaction of the guanamines, either before or after their application to the fiber, or both, and by suitable treatment the finish may be made wash-resistant. This is an important advantage of the invention, for my guanamine-containing finishes are then permanent in character and possess a long and effective life on the fiber.

Most of the higher alkyl guanamines used in practicing the present invention are light-colored crystalline solids having relatively high melting points and good stability against heat and discoloration. The unsubstituted members of the series have melting points in the range of about 75—150° C. while the corresponding mono-N-acyl derivatives have much higher melting points. On the other hand the melting points of the N-N'-diacyl compounds are considerably lower than the melting points of the corresponding unsubstituted guanamines and a wide range of com-

pounds of varying physical characteristics is therefore presented by the invention in its broader aspects. Most of the higher alkyl guanamines are soluble in hot mineral spirits, in glyceride oils and in xylene, but are insoluble or sparingly soluble in water. As a rule the compounds of my invention show increasing solubility in the above solvents with increasing chain length and with increased branching of the chain.

10 The higher alkyl guanamines as a class are compounds corresponding to the formula



15 in which R is a saturated or unsaturated aliphatic or cycloaliphatic group containing at least 7 carbon atoms attached to the triazine nucleus by a carbon-to-carbon bond. This group may be further substituted by halogen, hydroxy, alkoxy, oxyaryl, aryloxy, carboxylic, carbonyl, sulfonic, 20 amino, amido or other groups as will be subsequently explained, and any one or more of A, B and X may be H or any other substituent such as acyl, alkyl, cycloalkyl, aromatic and the like. A few representative compounds falling within 25 the above definition, and which may be applied to textile threads or fibers to vary the properties thereof in accordance with the present invention, are as follows:

30 (1) Representative long chain saturated or unsaturated aliphatic guanamines are octanoguanamine, decanoguanamine, lauroguanamine, myristoguanamine, palmitoguanamine, stearoguanamine, oleoguanamine, linoleoguanamine and similar higher alkyl guanamines obtained by the 35 reaction of biguanide or substituted biguanides with vegetal (animal and vegetable) oils, the fatty acids thereof or preferably the methyl esters of these fatty acids such as those obtained from olive oil, hydrogenated cotton seed oil, coconut oil, teaseed oil, peanut oil and the like. Usually 40 guanamines obtained from saturated higher fatty acids or from fatty acids having only a limited degree of unsaturation such as oleic acid are preferred in practicing the invention, as the more 45 unsaturated compounds are less stable to oxidation and to chlorine from laundry bleaches.

50 (2) Representative branched chain guanamines which may be used in practicing the invention are methyl-isoamylacetoguanamine, N-acyl acetoguanamines, beta - beta - di-n-propylpropionoguanamine, di-isobutylacetoguanamine, n-amyl-n-heptylacetoguanamine, di-n - heptylacetoguanamine, di-n-octylacetoguanamine, ethyl-n-butyacetoguanamine, ethyl - isoamylacetoguanamine, di-n-butylacetoguanamine, di-n-propylac-

etoguanamine, 4'-ethyl-2-octanoguanamine. Representative cycloaliphatic guanamines are those obtained, for example, by condensing naphthenic acids and their aliphatic esters with biguanide or substituted biguanides and similar condensation products of maleic acid or anhydride with tung oil and with terpenes, and ortho-carboxy-endomethylene-tetrahydrobenzoguanamine obtained by condensing "carbic" acid with an equimolecular quantity of biguanide.

(3) As has been noted above, the aliphatic radical R may be substituted by inorganic or organic substituents. Representative compounds of the first class suitable for textile finishing are alpha-alpha'-dichloro stearoguanamine, 9-10 dibromo stearoguanamine, 10-bromo decanoguanamine and salts of 10-sulfo decanoguanamine.

The guanamines used in practicing the present invention include those in which the aliphatic or cycloaliphatic radical R is interrupted by one or more substituents as well as compounds in which the carbon chain or ring is uninterrupted, for I have found that good results are obtainable with compounds of both types when the radical contains a total of at least seven carbon atoms. Thus, for example, beta-octadecylamino-propionoguanamine and stearylamino-acetoguanamine possess softening and waterproofing properties for textiles comparable to those of stearoguanamine, particularly when condensed with formaldehyde. Other compounds illustrative of the class of guanamines containing organic substituents are the higher alkoxyalkyl guanamines such as beta-octadecoxypropionoguanamine and beta-amyloxypropionoguanamine. Compounds representative of other groups that may be present are omega-carbomethoxy-pelargonoguanamine, omega-carbobutoxypelargonoguanamines, omega-carboxypelargonoguanamine, beta-N-dibutylcarbamyl-propionoguanamine, alpha-methoxy-beta-N-octylcarbamylpropionoguanamine.



beta-carboxy-beta-amyloxypropionoguanamine and omega-acetyl undecanoguanamine.

(4) As is pointed out in my copending application Serial No. 409,113, filed concurrently herewith, the presence of substituents on one or both of the amino groups of the guanamines is frequently of advantage in textile treatment, for these substituents may modify the solubilities of the compounds and their compatibility with resins, waxes, starches, gums and other ingredients of textile finishing compositions with which the guanamines may be employed. Representative N-substituted higher alkyl guanamines that have been prepared and tested are 4-N-phenyl-lauroguanamine, 4-N-butyl-2-(alpha-ethyl)hexano-guanamine, 4-N-octanoyl-octanoguanamine, 4-N-lauroyl-lauroguanamine, 4-N-stearoyl-stearoguanamine, 4-N-phenyl-stearoguanamine and di-substituted derivatives such as 4-N-phenyl-6-N-myristoyl-myristoguanamine and 4,6-N,N'-diacetyl decanoguanamine.

The above and other guanamines falling within the scope of the invention may be prepared by reacting biguanide or substituted biguanides with unsubstituted or substituted aliphatic and cycloaliphatic carboxylic acids and their esters and halides. When the acid halides are used the reaction usually proceeds smoothly upon simple admixture of the reagents in the presence of inert solvents, but when the esters are employed it is frequently desirable to carry out the reac-

tion in the presence of alkaline catalysts. Metal alcoholates are particularly useful for this purpose, and sodium methylate is the preferred catalyst. The condensation product is usually recovered by filtration and purified by recrystallization from methanol, other alcohols, acetone, methylethyl ketone, hot water or other suitable solvents. Many of the N-substituted guanamines may also be prepared from the corresponding unsubstituted guanamines by fusion with amine salts, preferably in the presence of a flux such as phenol and a condensation catalyst such as zinc chloride. N-acyl guanamines may be prepared in similar manner by heating the unsubstituted guanamine with an acid chloride or acid anhydride.

It is an important advantage of the higher alkyl guanamines falling within the scope of the present invention that they will combine with formaldehyde, acetaldehyde, butyraldehyde and other aldehydes to form condensation products, for it is in this form that they are most useful as finishing agents for textiles. When dispersible resins are desired it is usually advisable to employ guanamines containing at least two replaceable amino hydrogen atoms and to use rather mild conditions for the aldehyde condensation, such as by agitating the aldehyde and guanamine solution at 50-70° C. until the reaction is complete, and an inert solvent may be used to maintain the guanamine in a dispersed form at these temperatures. The resulting resin solutions which are first formed can usually be diluted with limited quantities of water, but upon continued heating or upon reaction at higher temperatures a hydrophobic resin is produced. Further polymerization is obtained upon heating the resin after its application to the textile fibers, and a permanent laundry-resistant waterproofing effect is obtained when the fiber is first impregnated with the resin in its water-dispersible stage and then subsequently heated to further cure the resin to the water-insoluble stage.

Although other aldehydes may be employed I prefer to condense the guanamines with formaldehyde, which may be used in the form of ordinary 37% formalin solutions, or as strong aqueous formaldehyde solutions of 40-50% strength stabilized by the addition of 4-10% of melamine, or as paraformaldehyde. At least one mole of formaldehyde for each mole of guanamine should be used, and in the case of N-unsubstituted guanamines at least two moles of formaldehyde should be employed. When higher formaldehyde ratios of the order of 6-8 moles or more for each mole of the guanamine are employed the condensation product is more easily dispersible in water.

The guanamine-formaldehyde condensation products are quite easy to obtain in the form of substantially monomolecular products; that is to say, as methylol guanamines. When lauroguanamine, stearoguanamine and other N-unsubstituted long chain guanamines are combined with formaldehyde under the mild conditions described above there is first obtained a hydrophilic syrup. Upon evaporation of the solvent or solvents under reduced pressure at 30-40° C. methylol guanamines are obtained which are soluble in hot mineral spirits, hot alcohols and hot xylene and which can be crystallized from these solvents upon cooling, and which are compatible with urea-formaldehyde, melamine formaldehyde and alkyd resins. These compounds can be alkylated by heating with primary alcohols such

as methanol, ethanol and butanol in the presence of small amounts of phosphoric acid, oxalic acid or hydrochloric acid with azeotropic distillation of the water of condensation and the resulting products may be applied to textiles from their solutions in organic solvents as creaseproofing agents and water-repellents.

Many of the higher alkyl guanamines are soluble in such organic solvents as acetone, toluene, dioxane and ethers of ethylene glycol and may be applied as such to textiles as softening agents. The aldehyde condensation products can also be applied as solutions in these and similar organic solvents. In addition to the dispersibility obtained by the use of mild temperature conditions during the condensations and by excess formaldehyde, referred to above, the condensation products can be dispersed in water containing equimolecular amounts of organic acid such as acetic, lactic and alpha-hydroxy isobutyric acids, and these acids will also act as curing accelerators for the resins after their application to the cloth. The resins are also solubilized by ammonia and other alkalis. Polymerization products obtained by heating glycidol and other 25 alcohols containing an ethylene oxide ring are also good dispersing agents.

Another class of agents that are particularly well suited for use as dispersing agents are aliphatic and cycloaliphatic substituted guanamines in which the alkyl radical contains a sulfonic group, such as omega-sulfodecanoguanamine or one or more carboxylic acid groups such as omega-carboxy-propionoguanamine, omega-carboxy pelargonoguanamine and the like. These 35 compounds in which the 2-aliphatic or cycloaliphatic substituent contains a hydrophilic group may be mixed with the guanamine resins to be solubilized in amounts of 5% to 15% or more, or they may be themselves reacted with the aldehyde either alone or in admixture with the other guanamines without losing their water dispersing properties. Another compound which aids in the water dispersal of the higher alkyl guanamine resins is the guanamine obtained by condensing biguanide with "Petrex," which is a diene condensation product of pinene with maleic anhydride.

Additional solubilizing and dispersing agents are also described and claimed in the copending application of Stiegler, Fluck and Thurston, Serial No. 409,114, filed concurrently herewith. As is pointed out in that application, such wetting and emulsifying agents as sodisopropyl naphthalene sulfonate, sodium lauryl sulfate, glycerine and other polyhydric alcohols, partially or completely neutralized sulfite cellulose liquor, sodium, ammonium and ethanolamine stearate, oleate and other higher fatty acid salts and ammonium caseinate may be used as dispersing agents for the preparation of textile finishing baths containing higher guanamines and guanamine-aldehyde condensation products.

In addition to the application of the higher alkyl guanamines and their aldehyde condensation products to textiles as the principal finishing agent these compounds may be applied in admixture with resins, gums, balsams and other binders that will give increased permanency to the finish. Thus, for example, urea-formaldehyde resins, melamine-formaldehyde resins, phenol-formaldehyde resins, alkyd resins or any other curing type of resin may be used to assist in binding the guanamine to the fiber. These additional binding agents can be used in consider-

able excess over the amount of guanamine resin, and the retention of the finish on the fiber after laundering is thereby greatly improved.

As has been stated above, one of the most useful methods of preparing textile treating baths containing higher alkyl guanamine compounds is with the aid of dispersing agents. A typical procedure of this kind, which may be used for applying any of the compositions of my invention to textiles, is as follows:

A solution of the higher alkyl guanamine-aldehyde resin is prepared in methanol, ethanol, isopropanol or other suitable solvent by heating with agitation. An aqueous dispersion of a resin, gum or other suitable binding agent is then prepared having a concentration suitable for application to the fiber; for example, a solution of 10-15 parts or more of water-soluble urea-formaldehyde resin or of methylated methylol melamine in sufficient water to make 100 parts. About 5-10 parts by weight of a 5% solution of a suitable dispersing agent such as sodium isopropyl naphthalene sulfonate is added to this bath and the alkyl guanamine resin solution is poured in with stirring while maintaining the temperature at about 115° F. A dispersion having an extremely fine particle size is thus obtained, to which a curing accelerator may be added to speed up the setting of the resin after its application to the fiber if desired. Four per cent based on the total resin solids of a mixture of 4 parts hexamethylene tetramine and 30 parts of diammonium phosphate has been used to advantage. The cloth to be treated is immersed in this bath and then passed through squeezing rolls adjusted to a tension such that the quantity of treating solution retained on the cloth is approximately equal to the weight of the fabric. The treated cloth is then dried at about 250° F. and heated for a short time at higher temperatures to cure the resin. A permanent and laundry-resistant waterproof finish is thereby imparted to the cloth.

It should be understood that the above described aqueous dispersion of higher alkyl guanamines in admixture with urea-formaldehyde and particularly methylated melamine-formaldehyde resins is not claimed as such in the present application. On the contrary, these dispersions and their application to textiles are claimed in the application of Stiegler, Fluck and Thurston, referred to above.

The invention will be illustrated in greater detail by the following specific examples, which show representative compositions included therein. It should be understood, however, that although these examples may describe in detail some of the more specific details of the invention they are given primarily for illustrative purposes and the invention in its broader aspects is not limited thereto.

#### Example 1

Stearoguanamine was prepared by reacting 150 parts by weight of biguanide and 300 parts of methyl stearate in a mixture of 500 parts of ethanol and 1088 parts of methanol having 23 parts of sodium dissolved therein. The mixture was agitated until homogeneous and then allowed to stand for about 65 hours, whereupon the precipitated condensation product was filtered. This product was purified by recrystallization from methyl ethyl ketone and an almost colorless product melting at 112-114° C. was obtained. Further purification by recrystallization gave a stearoguanamine melting at 116-117° C., but for

most purposes the product of lower melting point is satisfactory.

Decanoguanamine, n-octanoguanamine, 2'-ethylhexanoguanamine, lauroguanamine and myristoguanamine were prepared by substantially the same process and formaldehyde condensation products were obtained by agitating with 37% aqueous formalin solutions at 75-80° C. in the ratio of 3-8 moles formaldehyde for each mole of the guanamine for periods of time varying from about 25 hours to 3 hours depending upon the pH of the solution, the guanamine used, the stage of polymerization product desired, and whether the formalin was diluted with an organic solvent such as methanol or ethanol. In the presence of alcohol as a diluent and at pH values from about 7.0 to 9.0 the reaction times were much longer than in the absence of the diluent.

The preparation of a stearoguanamine-formaldehyde is typical, and is as follows:

A mixture of 42 parts by weight of stearoguanamine prepared by the above described process and 77.7 parts of 37% aqueous formaldehyde was heated at 70° C. for about 12 minutes with vigorous stirring. As the stearoguanamine became warm it softened and emulsified, and after 12 minutes the formaldehyde condensation product was obtained. When the reaction mixture was cooled with stirring the resin remained in the form of a stiff emulsion which could be dispersed in water, but evaporation of the water at 35-40° C. under reduced pressure gave a paste which hardened to a soft resin upon cooling and further dehydration.

#### Example 2

Equimolecular quantities of biguanide and sodium butyl sebacate were dispersed in methanol, thoroughly mixed, and allowed to stand for several days until precipitation of the condensation product was complete. The solid material was filtered, washed with methanol, and dried. The sodium salt of omega-carboxypelargonoguanamine was extracted from the condensation product with hot water and precipitated by addition of mineral acid to a pH of about 4.0. After purification by solution in alkali and reprecipitation with acid a pure product was obtained in the form of a white solid melting at 223-225° C.

35 parts by weight of the omega-carboxypelargonoguanamine was mixed with 60 parts of 37% formalin and the mixture was heated to 67° C. with continuous stirring. After 1.5 hours the original thick mixture became thinner and finally homogeneous, and upon stopping the agitator after 2 hours of heating the mixture separated into two liquid layers. Upon decanting the thin water layer and drying the resin at reduced pressure a viscous gum was obtained which was soluble in sodium hydroxide, ammonia, triethanolamine and other alkalies.

5 parts by weight of the resin were dissolved in 50 parts of dilute ammonium hydroxide solution and cotton cloth was padded in the bath so prepared. The cloth was then squeezed until the resin content was 5% on the weight of the fiber and then placed in a mordanting bath of aluminum sulfate to precipitate the aluminum salt on the fiber. The cloth was then dried in an oven whereupon it was found to possess good water repellent properties.

#### Example 3

10 parts by weight of stearoguanamine and 20 parts of omega-carboxypelargonoguanamine were combined with 46 parts of 37% formalin by the

procedure described in Example 2. After heating at 70° C. for 2.5 hours the thick resin was dried to give a solid which was soluble in ammonia.

Impregnating baths were prepared by dissolving the mixed resin in ammonia in varying concentrations, and the finish was applied to cotton percale and to spun rayon dress goods. The impregnated samples were dried 5 minutes at 250° F. and cured 3 minutes at 300° F. without the addition of a curing accelerator to the bath. Soaps were made using 0.5% soap solution containing 0.2% of soda ash in an electric washing machine for 1 hour at 160° F., followed by thorough rinsing. Dry cleaning tests were carried out by agitating the samples in trichlorethylene for 30 minutes.

1% and 10% of the finish was applied to cotton percale. The 1% sample, before soaping, possessed a soft hand and a tendency to repel water; the hand of the 10% sample was somewhat harsher and the fabric showed good water-repellent properties. Both the 1% and the 10% sample showed good resistance to soaping and to dry cleaning, and both samples retained their water-repellent properties after these tests. The results on spun rayon were similar to those on cotton, except that the finish was livelier.

#### Example 4

1.5 parts by weight of the stearoguanamine resin described in Example 1 were dissolved in methanol and emulsified in 100 parts of a solution containing 10 parts of the methyl ether of trimethylol melamine, 0.6 part of isopropyl naphthalene sulfonate and 4.6 parts of a curing accelerator. 80x80 cotton percale was padded in this bath, passed through squeeze rolls set to retain an equal weight of the finishing composition on the cloth, dried, and heated to cure the finish on the fiber. The cloth was then found to have excellent water-repellency, and could be held under a running stream of tap water without becoming wet.

Compositions similar to the above were prepared using formaldehyde condensation products of myristoguanamine, lauroguanamine, caproguanamine and capryloguanamine instead of stearoguanamine. Cotton cloth impregnated with these compositions, dried and cured also possessed good water-repellency.

#### Example 5

The hydrophobic properties of cloth treated with higher alkyl guanamines in accordance with the present invention were determined quantitatively by a standard spray test, which is applied as follows:

A six-inch square of cloth treated with the waterproofing agent, dried and cured is weighed and then suspended 10 inches from a horizontal spray nozzle supplied with water at 70° F. under a head of exactly 6 feet. The cloth is sprayed for 1 minute, during which time 1½ gallons of water are discharged through the nozzle, drained for 10 seconds, rolled between pieces of absorbent paper to remove surface water, and again weighed. The increase in weight is expressed as per cent water absorbed, based on the original dry weight of the cloth.

In order to measure the resistance of the finish to laundering, samples of the treated cloth were washed in an 0.5% soap solution at 160° F. 30 minutes, rinsed and dried, and again subjected to the spray test. The samples were then

washed again for a total of 3.5 hours. The higher water absorption values of the first spray tests are explained by the presence of partially reacted resin components and accelerator on the cloth which would tend to absorb water.

The finished samples of cloth described in Example 4 were subjected to this test with the following results:

| Compound         | Carbon atoms<br>in side chains | Percent water absorbed after washing |          |
|------------------|--------------------------------|--------------------------------------|----------|
|                  |                                | 0.5 hr.                              | 3.5 hrs. |
| Stearoguanamine  | 17                             | 33.1                                 | 25.3     |
| Myristoguanamine | 13                             | 33.6                                 | 29.4     |
| Lauroguanamine   | 11                             | 35.2                                 | 32.4     |
| Caproguanamine   | 9                              | 37.6                                 | 35.2     |
| Octanoguanamine  | 7                              | 40.4                                 | 41.7     |

#### Example 6

An alkyd resin of high acid number (resin A) was prepared by the simultaneous reaction of 190 parts by weight of phthalic anhydride, 101 parts of glycerine and 106.5 parts of cottonseed fatty acids. After reacting these ingredients and holding for the desired viscosity the acid number of the resin was 60.

An alkyd resin of low acid number (resin B) was prepared by reacting 183 parts by weight of phthalic anhydride, 100 parts of glycerine and 235 parts of castor oil at 425-450° F. until a resin having an acid number of 6-8 was obtained. This resin was cut with 115 parts of butanol to 78% solids.

Resin A was cut to 80% solids by the addition of toluene and 67.5 parts by weight of this 80% solution were taken. 163.5 parts by weight of the resin B solution were added and the mixture was warmed to 40° C. and stirred for about 10 minutes, or until a homogeneous mixture was obtained. 35 parts by weight of the stearoguanamine-formaldehyde resin of Example 1 were stirred into 274 parts by weight of a 50% solution of a butylated urea-formaldehyde resin in a mixture of equal parts of butanol and xylene and the resulting solution was then added to the alkyd resin solution and the mixture was cooled to 30° C. and stirred for an additional 10 minutes or until the entire mixture was homogeneous in character.

An ammonium caseinate solution was prepared in the following manner: 39 parts by weight of casein were soaked in 440 parts of water for 1/2-3 hours at room temperature, or until the casein was sufficiently swollen, and the mixture was then heated to 50-80° C. to insure uniform hydration. After cooling to 40-50° C. an ammonium hydroxide solution was added in amounts sufficient to obtain a uniform dispersion of the casein. Experience with emulsifying agents of this type has shown that amounts of 28% ammonium hydroxide ranging from 20 to 26 parts by weight are satisfactory for this purpose, the exact amount depending upon the final pH desired in the finished emulsion. After all the casein was dissolved by the ammonium hydroxide solution additional water was added to make a total of 505 parts by weight.

The mixture of high acid number alkyd resin, low acid number alkyd resin, butylated urea-formaldehyde resin and stearoguanamine resin was agitated vigorously at 30° C. and the solution of emulsifying agent was slowly added. Addition of the entire 505 parts of the emulsifier was made over a period of about 40 minutes,

after which agitation of the mixture was continued for an additional 30 minutes or until a completely uniform emulsion was obtained. This emulsion was perfectly stable upon storage and could be easily diluted with water without separation.

All wool fabric was padded in a sizing bath containing 3 gallons of the above emulsion to 100 gallons of water. The impregnated fabric was dried under tension to prevent shrinkage for 7 minutes at 250° F. The dried fabric was found to possess the same softness as that of the original material, but was much firmer, and possessed good water-repellent properties.

Equally good results were obtained when the butylated urea-formaldehyde was replaced by an equal quantity of butylated melamine-formaldehyde resin prepared by condensing melamine with formaldehyde in the ratio of about 1:5 in the presence of an excess of n-butanol and heating with distillation of water until an anhydrous product is obtained.

#### Example 7

35.4 parts by weight of phenyl biguanide and 60 parts by weight of methyl stearate were added to a solution of 4.6 parts by weight of sodium in 160 parts of methanol to which 50 parts of the butyl ether of ethylene glycol (Butyl Cellosolve) had been added. The mixture was allowed to stand at room temperature for 24 hours after which it was evaporated to dryness at reduced pressure. The product was extracted with carbon tetrachloride, the solution evaporated to dryness, and the solids recrystallized from methanol. The product was a white crystalline solid which was identified as 4-N-phenyl stearoguanamine.

A representative sample of the crystalline product was converted into a resin by reaction with 40 formaldehyde in the ratio of 5 moles of aldehyde for each mole of the 4-N-phenyl stearoguanamine. The reaction was carried out by dissolving the guanamine in methanol with the addition of heat, adding formaldehyde which had been neutralized to a pH of 8.0 and agitating for about 60 minutes at 70° C. The product had a melting point of 64-65° C., and could be recrystallized from methanol as a definite methylol guanamine containing 0.6 mole of formaldehyde per mole of guanamine. The compound was found to be a plasticizer for urea-formaldehyde textile finishing compositions used for creaseproofing purposes, and was suitable for use in admixture with such compounds.

#### Example 8

Ethyl beta-octadecoxy-propionate was prepared from octadecoxy propionitrile by refluxing the nitrile with concentrated sulfuric acid in the presence of 95% ethanol for 7 hours. The product was purified by extraction with chloroform and filtration to remove ammonium sulfate and the filtrate was neutralized with sodium bicarbonate, washed with water and dried.

A mixture containing 92.5 parts by weight of the ethyl beta-octadecoxy-propionate, 25 parts of biguanide, 400 parts of methanol, and 400 parts of ethanol was stirred at room temperature for 15 hours and then allowed to stand for 4 days. The resulting guanamine was removed by filtration and after recrystallization from acetone was found to have a melting point of 108-110° C.

A representative sample of the beta-octadecoxypropionoguanamine was converted to the methylol compound by reaction with 37% aque-

ous formaldehyde solution having a pH of 8.2 in the ratio of 6 moles of formaldehyde for each mole of the guanamine. The reaction was carried out in the methanol solution by heating the mixture at 70° C. for 45 minutes. The product when dispersed in water by the addition of acetic acid was found to be an excellent waterproofing agent for cotton cloth, cellulose acetate cloth, and other textile fibers.

A textile treatment bath was prepared containing 1.5 parts by weight of the above described guanamine resin and 10 parts by weight of a lower-primary alcohol-reacted melamine-formaldehyde resin. When cotton cloth was padded in this bath, dried, and cured at suitable temperatures it showed waterproofing properties comparable to those of the best waterproofed cotton fabrics now on the market.

#### Example 9

16.8 parts of 4-N-octanoyl-octanoguanamine was stirred into a mixture of 20 parts of 37% aqueous formaldehyde neutralized to pH 8 with triethanolamine, and 100 parts of isopropanol. The mixture was heated to reflux, 100 parts of butanol were added, and the refluxing was continued for 40 minutes. After this time the isopropanol was distilled and the product was cooled and filtered to remove a small amount of uncombined guanamine.

The filtrate was a clear syrup containing 18% of the octanoguanamine resin by weight. 100 parts of this syrup were dispersed in 1000 parts of an aqueous solution containing 10% of methylated methylol melamine, 5 parts of a mixture containing 88% diammonium phosphate and 12% of hexamethylene tetramine and 6% of sodium isopropyl naphthalene sulfonate. 80 x 80 cotton percale was padded in this solution, dried at 250° F. and cured 4 minutes at 300° F., after which treatment it was found to possess improved softness and water-repellency.

#### Example 10

Aminoacetoguanamine was prepared by reacting a solution of 70 parts by weight of glycine ethyl ester hydrochloride in 200 parts of methanol, 13.8 parts of metallic sodium in 200 parts methanol, and a solution of 60.5 parts of biguanide in 175 parts methanol. The sodium methylate solution was first added to the glycine ester salt, the resulting sodium chloride filtered off, and the filtrate added to the biguanide solution.

68 parts by weight of stearyl chloride was dissolved in 50 parts of dioxane and slowly added to a suspension of 28 parts of aminoacetoguanamine in 200 parts of pyridine while maintaining the temperature below 20° C. The reaction mixture was allowed to stand for 5 hours and was then refluxed for one-half hour, after which it was poured into ice water and the product recovered and recrystallized. The stearylaminoacetoguanamine so prepared was a light tan solid which softened at 120° C. and was completely fused at 174° C. The product was condensed with formaldehyde, using 6 moles of 37% aqueous formaldehyde solution for each mole of the stearylaminoacetoguanamine. The formaldehyde was adjusted to a pH of 8.0 and added to a suspension of the guanamine in methanol and the mixture was heated to 75° C. and agitated at this temperature for 30 minutes. The resulting resin was applied as a water repellent to spun rayon challis. An emulsion was prepared in the man-

ner previously described using 1.5% of the guanamine and 10% of methylated methylol melamine, based on the total weight of the solution, and 6% of curing accelerator, based on the amount of resin. After drying at 250° F. and curing for 4 minutes at 280° F. the cloth was soaped 30 minutes, rinsed and dried, and subjected to the spray test. It was found that only 39.6% of water was taken up by the fabric.

#### Example 11

123 parts of 37% aqueous formaldehyde solution having a pH of 8.5 are mixed with 100 parts of ethyl-n-butylacetoguanamine and the mixture is heated at 60-100° C. for 1-3 hours, thus producing a clear, aqueous syrup.

58 parts of 37% formalin having a pH of about 4-5 are mixed with about 100 parts of ethyl-isoamylacetoguanamine and heated under reflux at 70-90° C. for about 3 hours, thereby producing a clear aqueous syrup.

100 parts of impure di-n-butylacetoguanamine and 68 parts of 37% formalin having a pH of 4-5 are mixed and refluxed at 60-90° C. until a clear syrup is obtained, requiring about 1-4 hours. Similarly other guanamines having branched chain radicals containing at least 7 carbon atoms may be condensed with aldehydes such as formaldehyde in the same general manner as set forth in the above examples. Mixtures of the guanamines with melamine, urea, or mixtures of melamine and urea, when condensed with formaldehyde or other aldehydes produce resinous condensation products having desirable properties as the guanamines appear to exert a plasticizing action on the melamine and urea condensation products.

The aqueous resinous syrups prepared according to my invention have a wide variety of applications in the treatment of textiles. They may be applied in the form of solutions, dispersions or emulsions to produce a wide variety of effects. Creaseproofing, the production of mat finishes, waterproofing, glazing chintz, rendering textiles water-repellent, etc., are a few of the textile applications.

My guanamine-aldehyde condensation products are also of use in affixing dyes to fabrics, particularly those containing cellulose and the cellulose derivatives such as cellulose acetate, cellulose propionate, ethyl cellulose, etc. Dyes, lakes and pigments may be mixed with my guanamine-aldehyde condensation products and upon heating the mixture, insoluble materials are obtained. Furthermore, dyes, lakes and pigments, 55 may be applied to substrata either before or after an application of a solution, dispersion or emulsion containing my guanamine-aldehyde condensation products. Upon application of heat, the dyes, lakes, or pigments are affixed to the substrata by means of the insoluble guanamine-aldehyde condensation products.

Generally in the treatment of textiles, it has been found preferable to use aqueous syrups containing my guanamine-aldehyde condensation products and if this be done, various water-soluble adjuncts may be admixed therewith, e. g., starch, gum tragacanth, the alginates, casein, etc. Suitable softeners may be included in the compositions. In some instances, it is especially desirable to use emulsions of my guanamine-aldehyde condensation products, particularly in textile printing. Wetting agents may be incorporated with my products for special purposes in the treatment of textiles.

75 This application is a continuation-in-part of

my copending application Serial No. 331,810, filed April 26, 1940.

What I claim is:

1. A method of finishing textiles which comprises the step of applying thereto a finishing agent containing a water-insoluble guanamine having a member of the group consisting of aliphatic and cycloaliphatic radicals containing at least seven carbon atoms directly attached to the 2-carbon atom thereof by a carbon-to-carbon bond and then heating the textiles to dry and set the finish on the fibers.
2. A method of finishing textiles which comprises the step of applying thereto a finishing agent containing an aldehyde condensation product of a water-insoluble guanamine having a member of the group consisting of aliphatic and cycloaliphatic radicals containing at least seven carbon atoms directly attached to the 2-carbon atom thereof by a carbon-to-carbon bond and then heating the textiles to dry and set the finish on the fibers.
3. A method of finishing textiles which comprises the step of applying thereto a finishing agent containing a formaldehyde condensation product of a water-insoluble guanamine having a member of the group consisting of aliphatic and cycloaliphatic radicals containing at least seven carbon atoms directly attached to the 2-carbon atom thereof by a carbon-to-carbon bond and then heating the textiles to dry and set the finish on the fibers.
4. A method of finishing textiles which comprises applying thereto a finishing agent containing a water-insoluble guanamine having a member of the group consisting of aliphatic and cycloaliphatic radicals containing at least seven carbon atoms directly attached to the 2-carbon atom thereof by a carbon-to-carbon bond together with a binder therefor and then subjecting the fibers to heating to set the finishing agent on the fiber.
5. A method of finishing textiles which comprises applying thereto a finishing agent containing a water-insoluble guanamine in which the 2-carbon atom is connected by a carbon-to-carbon bond with a member of the group consisting of aliphatic and cycloaliphatic radicals containing at least seven carbon atoms together with a curable heat-curing resin other than a guanamine-formaldehyde resin and then heating the textiles to set the finishing agent thereon.
6. A method of finishing textiles which comprises applying thereto a finishing agent containing a water-insoluble guanamine in which the 2-carbon atom is connected by a carbon-to-carbon bond with a member of the group consisting of aliphatic and cycloaliphatic radicals containing at least seven carbon atoms together with a curable heat-curing alkyd resin and then heating the textiles to set the finishing agent thereon.
7. A method of finishing textiles which comprises the step of applying thereto a finishing agent containing a water-insoluble guanamine in which the 2-carbon atom is connected by a carbon-to-carbon bond with an aliphatic radical containing at least seven carbon atoms and then heating the textiles to dry and set the finish on the fibers.
8. A method of finishing textiles which comprises the steps of preparing a liquid finishing composition containing a dispersion of a water-insoluble guanamine in which the 2-carbon atom is connected by a carbon-to-carbon bond with an aliphatic radical containing at least seven carbon atoms, impregnating the textiles with said finishing composition, and heating the impregnated textiles to dry the same and set the finish on the fibers thereof.
9. A method of finishing textiles which comprises the steps of preparing a liquid finishing composition comprising an aqueous dispersion of a water-insoluble guanamine in which the 2-carbon atom is connected by a carbon-to-carbon bond with an aliphatic radical containing at least seven carbon atoms, impregnating the textiles with said finishing composition, and heating the impregnated textiles to dry the same and set the finish on the fibers thereof.
10. A method of finishing textiles which comprises the steps of preparing an aqueous dispersion containing a water-insoluble guanamine in which the 2-carbon atom is connected by a carbon-to-carbon bond with an aliphatic radical containing at least seven carbon atoms, said dispersion also containing as an emulsifying agent a water-soluble guanamine containing an aliphatic radical that is substituted by a member of the class consisting of sulfonic and carboxylic acid groups, impregnating the textiles with said dispersion, and heating the impregnated textiles to dry the same and set the finish on the fibers thereof.
11. A method of finishing textiles which comprises the step of applying thereto a finishing agent containing a 2-alkyl guanamine in which the 2-alkyl group is a hydrocarbon chain containing at least seven carbon atoms and then heating the textiles to dry and set the finish on the fibers.
12. A method of finishing textiles which comprises the step of applying thereto a finishing agent containing a 2-alkyl guanamine in which the 2-alkyl group is a hydrocarbon chain containing nine to seventeen carbon atoms and then heating the textiles to dry and set the finish on the fibers.
13. A method of finishing textiles which comprises the step of applying thereto a finishing agent containing a formaldehyde condensation product of a 2-alkyl guanamine in which the 2-alkyl group is a hydrocarbon chain containing at least seven carbon atoms and then heating the textiles to dry and set the finish on the fibers.
14. A method of finishing textiles which comprises the step of applying thereto a finishing agent containing a formaldehyde condensation product of a 2-alkyl guanamine in which the 2-alkyl group is a hydrocarbon chain containing nine to seventeen atoms and then heating the textiles to dry and set the finish on the fibers.
15. A method of finishing textiles which comprises the step of applying thereto a finishing agent containing stearoguanamine and then heating the textiles to dry and set the finish on the fibers.
16. Textiles characterized by improved water-repellency and having the individual fibers thereof coated with a cured finishing composition containing a water-insoluble guanamine having a member of the group consisting of aliphatic and cycloaliphatic radicals containing at least seven carbon atoms directly attached to the 2-carbon atom thereof by a carbon-to-carbon bond said textiles having been finished by the method of claim 3.

JACK T. THURSTON.